

1

3,070,484

PROCESS FOR THE PRODUCTION OF PULPS  
FROM LIGNIN-CONTAINING CELLULOSE  
MATERIAL

Anton Rudolf Wacek, Graz, Austria, assignor to Kimberly-Clark Corporation, Neenah, Wis., a corporation of Delaware

No Drawing. Filed Sept. 2, 1959, Ser. No. 837,596  
Claims priority, application Austria Sept. 5, 1958

7 Claims. (Cl. 162—23)

This invention relates to a process for the production of pulps from lignin-containing cellulose material by chemical or semi-chemical digestion of such material and has as its principal object the reduction of the degradation which normally accompanies such processes.

In conventional chemical digestion processes more or less severe degradation of the cellulose occurs, as is evident by the reduction in the original value for the molecular weight or the average degree of polymerisation (D.P.) of the cellulose. In general, the molecular weight or average D.P. of the cellulose drops to about one fifth of the original value. It has previously been assumed that this degradation is due to too long a cooking treatment, to the air present in the pores of the cellulosic material being digested and/or to mechanical wear and tear on the cellulose.

Many attempts have been made to eliminate or reduce the degradation which occurs during digestion but without any substantial degree of success. Thus, for example, experimenters have tried to accelerate the penetration of the cooking liquor into the comminuted cellulosic material, particularly in the case of wood chips, by increasing or decreasing the pressure used; by the use of changing pressure and evacuation; by the use of different temperatures, as well as by vaporization (see for example Das Papier, 11, page 14 (1957); Norwegian Patent No. 54,053; Finnish Patent No. 17,002; and U.S. Patent No. 2,072,776). It has also been proposed to digest the material with caustic soda of various concentrations in an atmosphere of hydrogen, using for example a preimpregnation process (Austrian Patent No. 72,881). In other known processes preimpregnation of the material is effected at a reduced pressure (U.S. Patent No. 1,025,336) or is effected under pressure before the material has reached a temperature above 110° C. (U.S. Patent No. 1,790,260). According to a still further process, the crude material is subjected to the action of the digesting agents after pre-treatment with anaerobic bacteria under pressure (German Patent 235,852), or wood and other fibrous plant materials in a comminuted state are surrounded with gas, e.g. carbon dioxide, hydrochloric acid gas or sulfur dioxide, for the purpose of dissolving out lignin and similar incrustations and are then shaken with concentrated sulfuric acid at room temperature and without pressure (German Patent No. 441,392). The object of these processes was, on the one hand, to obtain a better impregnation of the material and, on the other hand, to shorten the actual digestion process so as to obtain a greater through-put of the cookers or disintegrators. In addition, the degrading effect of the digestion was ascribed to the action of the air remaining in the pore spaces of the cellulosic material and it was hoped by preimpregnation to eliminate this air. These attempts, as has previously been stated, have not been outstandingly successful particularly when the cellulosic material is subjected before or during the chemical action of the digesting agent to mechanical treatment such as transport of the material or agitation or mechanical comminution during the cooking (see "Cellulose Chemie," 16, page 41 (1935), and Das Papier, 10, page 4 (1956)).

I have found that neither the extent of impregnation of

2

the cellulosic material (preimpregnation) nor the air or oxygen in the pores of the material, nor the mechanical treatment before or during the digestion is responsible for the main drop in the average D.P. of the cellulose. I have found that the primary cause of the degradation of the cellulose is the oxygen content of the gas space above the digestion liquor. Specifically, I have found that when wood chips are digested with bisulfite in the usual manner the digestion liquor always becomes dark or even black on rapid heating regardless of whether the chips have been previously impregnated or not if the chips come into contact with the oxygen-containing gas atmosphere in the cooker or autoclave. By contrast, when the air present in the cooker or autoclave is replaced by inert gas, such for example as nitrogen or carbon dioxide, the cellulosic material can be heated in a few minutes to the digestion temperature, even without preimpregnation of the material and without the liquor turning black.

I have further found that provided the chips or other lignin containing cellulosic material are treated with the digesting liquor while avoiding all contact of the cellulosic material with oxygen-containing gas, the liquor does not turn black and further the degree of degradation of the cellulose is considerably reduced. Thus the chips or other material may be so treated that throughout the digestion they are wholly immersed in the liquor.

Further, if the atmosphere above the digestion liquor, instead of being pure nitrogen or pure carbon dioxide, contains up to about 2% (the value varies somewhat with the nature of the cellulosic material) of oxygen the same effect, namely avoiding blackening and avoiding severe degradation of the cellulose, is obtained. Increase in the oxygen content of the inert gas to 5% brings about a slight browning of the material, while an increase to about 10% causes blackening of the cooking liquor and darkening of the cellulosic material.

According to the present invention, therefore, pulps are produced from lignin-containing cellulosic materials by digesting them with a cooking liquor while preventing contact of the cellulosic material with external gas containing more than 5% of oxygen. The term "external gas" is used in this specification to connote gas in contact with the outside of the cellulosic material and/or in contact with the cooking liquor and is used to exclude the gas contained in the pores of the material since I have determined that the presence of oxygen in the pores of the cellulosic material exercises no significant effect on the darkening of the cellulose, the blackening of the cooking liquor or the degradation of the cellulose.

While steps may be taken as described above to ensure that the wood or other cellulosic material remains completely immersed in the cooking liquor throughout the digestion process, it is preferable according to the present invention to fill the remainder of the digestor with inert gas.

The sulfite process is customarily used to obtain the whitest cellulose and to obtain the highest quality of cellulose. Accordingly, the process of the present invention is particularly valuable in relation to the sulfite digesting process. It may, however, equally well be used in the alkali process or in the sulfate process, it being understood that the latter two processes even with the present invention will not give such high quality cellulose as the sulfite process. The invention further includes both the customary sulfite process using bisulfite with free sulfur dioxide and also the so-called "neutral sulfite" process.

As is usual when employing an acid sulfite process any suitable soluble bisulfite may be used together with free sulfur dioxide, for example bisulfites of the alkali or alkaline earth metals or ammonia, e.g. sodium, potassium, ammonium, calcium and magnesium bisulfites.

The ratio of total  $\text{SO}_2$  to combined  $\text{SO}_2$  may be adjusted as is usual in the art.

I have further determined that given the conditions of the present invention the cellulosic material may be disintegrated or comminuted either before or during the digestion process without seriously degrading the cellulose. Further, the invention can be used in a continuous digestion process wherein the cellulosic material is pressed against a sieve or strainer and the liquor carrying additional cellulosic material gradually forced through the pad of chips or other cellulose.

Following on the digestion process of the invention wherein contact of the cellulosic material with oxygen is rigorously excluded, I find it advisable to exclude oxygen in any process of transferring of the cellulosic material from one piece of apparatus to another. Again, in defibering the pulp or otherwise treating the pulp while in contact with the liquor at fairly high temperature, it is advisable to exclude air or oxygen. Again this may be achieved by ensuring that the cellulosic material is continuously submerged in the liquor or alternatively the cellulosic material may be blanketed with inert gas.

By the process of the present invention good quality cellulose of high D.P. may be obtained. e.g. in the case of processes not using mechanical disintegration, D.P.'s of 1200 or above and in the case of processes using mechanical disintegration D.P.'s of 900 and above. Inasmuch as using the process of the present invention, previous comminution of the cellulosic material does not entail any severe drop of the D.P., the invention permits

of the use of sawdust as a raw material. Using sawdust it is generally necessary to stir or agitate during the digestion process.

Normally a sulfite digestion process operates at a temperature of about 130-140° C. or in the case of requiring highly purified pulps at a temperature up to 150° C. Higher temperatures are not possible in conventional processes because of the severe degradation and loss of cellulose which occur. Using the process of the present invention it is possible to cook at temperatures up to about 200° C. with consequent reduction in the cooking time. Furthermore, since according to the present invention preimpregnation of the cooking liquors is unnecessary, or at least produces little or no advantage, such preimpregnation may be omitted, again with resultant shortening of the total processing time.

The following examples illustrate the invention but do not limit it in any way. In the examples where grinding is carried out during the digestion a milling autoclave of the type shown in FIGURE 1 on page 5 of the article in Das Papier, vol. 10 (1956), was used. Where in the examples preimpregnation is used the method is that customarily used in the art, namely evacuation of the autoclave containing the cellulosic material followed by sucking in the cooking liquor, the process being repeated as many times as required. The D.P. of the products was determined by the Kraemer method (Industrial and Engineering Chemistry, vol. 30, page 1200 (1938)) and lignin was determined by the Tappi

Table 1

| Gas above liquor                        | Oxygen           |     |     |            | Nitrogen   |           |           |            |
|-----------------------------------------|------------------|-----|-----|------------|------------|-----------|-----------|------------|
|                                         | 56               | 56a | 56b | Mean value | 55         | 55a       | 55c       | Mean value |
| D.P.                                    | Not measurable   |     |     |            | 1,264      | 1,252     | 1,269     | 1,262      |
| Lignin content (in percent)             | 33.5             | 35  | 34  | 34.8       | 0.6        | 0         | 3.2       | 1.2        |
| Yield (in percent)                      | 60               | 62  | 63  | 61.6       | 50.8       | 49.5      | 52        | 50.8       |
| Defibering properties                   | Does not defiber |     |     |            | Very good  | Very good | Very good |            |
| Appearance of material and spent liquor | Black            |     |     |            | White      |           |           |            |
| Fiber structure                         | Destroyed        |     |     |            | Maintained |           |           |            |
| pH (of spent liquor)                    | 0.7              | 0.7 | 0.8 | 0.7        | 1.8        | 1.8       | 1.8       | 1.8        |

Table 2

| Gas above liquor            | Nitrogen        |       |       |            | Carbon dioxide  |      |      |            | Oxygen       |      |            |
|-----------------------------|-----------------|-------|-------|------------|-----------------|------|------|------------|--------------|------|------------|
|                             | 53              | 53a   | 53b   | Mean value | 54              | 54a  | 54b  | Mean value | 52           | 52a  | Mean value |
| D.P.                        | 1,053           | 1,028 | 1,070 | 1,050      | 949             | 980  | 919  | 949        | 425          | 641  | 533        |
| Lignin content (in percent) | 14.8            | 13.6  | 10.8  | 13.1       | 11.3            | 12.6 | 11.1 | 11.6       | 25.6         | 29.8 | 27.7       |
| Yield (in percent)          | 60              | 63.3  | 62    | 62         | 64.1            | 61.9 | 61.9 | 62.7       | 83           | 88   | 85         |
| Defibering properties       | Very good       |       |       |            | Very good       |      |      |            | Pulverulent  |      |            |
| Appearance of material      | Yellowish-white |       |       |            | Yellowish-white |      |      |            | Brown powder |      |            |
| Fibre structure             | Maintained      |       |       |            | Maintained      |      |      |            | Destroyed    |      |            |
| pH (of spent liquor)        | 1.8             | 1.8   | 1.8   | 1.8        | 1.6             | 1.4  | 1.5  | 1.5        | 1.2          | 0.8  | 1.0        |

method. In all cases whole knot-free wood was used in the form of chips.

#### EXAMPLE I

This example illustrates digestion using different gases above the digestion liquor without grinding during digestion.

The wood chips were previously impregnated with sodium bisulfite liquor containing 50 grams per litre of total  $\text{SO}_2$  and 10 grams per litre of combined  $\text{SO}_2$ . The ratio of chips to liquor was 1:7. After preimpregnation of the chips in the autoclave and bringing the liquor up to level, the autoclave was closed and the temperature brought as rapidly as possible to 150° C. The cooking time was 10 hours. The results were obtained as shown in Table 1.

#### EXAMPLE II

Further trials were carried out using the conditions of Example I with the exception that grinding was carried out continuously throughout the digestion process and the cooking time was 5 hours. The results obtained are shown in Table 2.

Comparison of the results obtained in Examples I and II using nitrogen as the inert gas above the digestion liquor shows that simultaneous grinding reduces the D.P. somewhat and also considerably reduces the time taken in digestion. In all cases using inert gas the D.P. is maintained at a commercially acceptable value.

#### EXAMPLE III

This example illustrates the negligible effect of gas in the pores of the wood chips. It compares the digestion under oxygen of wood chips containing nitrogen in the pores with the digestion under nitrogen of wood chips containing oxygen in the pores. The air in the pores in the former case was displaced by repeated evacuation in the autoclave and filling with nitrogen. In each case the cooking liquor was the same as in Example I, the cooking time was 10 hours, the cooking temperature 150° C. and the ratio of wood chips to cooking liquor was 1:7. The chips were not preimpregnated with the cooking liquor. The results are as follows:

6  
Table 3

| 5  | Trial number                | Gas above liquor |                  |            | In cooker space: Oxygen<br>In the pores: Nitrogen |      |            | In cooker space: Nitrogen<br>In the pores: Oxygen |       |            |
|----|-----------------------------|------------------|------------------|------------|---------------------------------------------------|------|------------|---------------------------------------------------|-------|------------|
|    |                             | 58               | 58a              | Mean value | 57                                                | 57a  | Mean value | 57                                                | 57a   | Mean value |
| 10 | D.P.                        |                  | Not measurable   |            |                                                   |      |            | 1,996                                             | 1,942 | 1,969      |
|    | Lignin content (in percent) | 36.5             | 35.2             | 35.8       | 3.7                                               | 10.9 |            |                                                   |       | 7.3        |
| 15 | Yield (in percent)          | 62.4             | 63               | 62.7       | 53.9                                              | 60   |            |                                                   |       | 57         |
|    | Defibering properties       |                  | Does not defiber |            |                                                   |      |            | Very good                                         |       |            |
| 20 | Appearance of material      |                  | Black            |            |                                                   |      |            | White                                             |       |            |
|    | Fiber structure             |                  | Destroyed        |            |                                                   |      |            | Maintained                                        |       |            |
|    | pH (of spent liquor)        | 0.7              | 0.7              | 0.7        | 1.7                                               | 1.8  |            |                                                   |       | 1.75       |

- 25 These trials demonstrate conclusively that the presence of oxygen in the pores exercises no substantial degrading action on the cellulose while the presence of oxygen in the space above the cooking liquor reduces the D.P. to a value at which it cannot be measured.
- 30 The results obtained in trials 57 and 57a of Table 3 may be compared with the results obtained in trials 55, 55a and 55c of Table 1 in Example I. The only difference between the conditions in the two sets of trials is that in Table 1 preimpregnation is used whilst in Table 3
- 35 there is no preimpregnation. It will be seen that very short extension of the cooking time of the trials of Table 3 gives equivalent results to those obtained in Table 1. This very short increase in cooking time is more than offset by the time used for impregnation in Example I.

40

#### EXAMPLE IV

This example demonstrates that much higher cooking temperatures may be used in the present process than in conventional processes. The conditions are identical with those used in Example I (using nitrogen above the cooking liquor) with the exception of the cooking temperature which was 200° C. and the cooking time which varied from 1½ to 2½ hours. The results obtained are as follows:

Table 4

| Digestion time in hours     | 1½         |       |       |       |            | 1¾         |      |            |      |     | 2               |      |      |            |      | 2½                 |      |      |      |            |
|-----------------------------|------------|-------|-------|-------|------------|------------|------|------------|------|-----|-----------------|------|------|------------|------|--------------------|------|------|------|------------|
| Trial number                | 74         | 74a   | 74b   | 74c   | Mean value | 80         | 80a  | Mean value | 73   | 73a | 73b             | 73c  | 73d  | Mean value | 78   | 78a                | 78c  | 78f  | 72   | Mean value |
| D.P.                        | 1,062      | 1,039 | 1,032 | 1,033 | 1,046      | 956        | 955  | 955        | 859  | 955 | 920             | 997  | 899  | 926        | 498  | 526                | 405  | 653  | 532  | 523        |
| Lignin content (in percent) | 21.8       | 20.7  | 20.4  | 19.2  | 20.5       | 16.8       | 14.5 | 15.6       | 16.4 | 16  | 16.3            | 16.3 | 16.9 | 16.4       | 4    | 5.2                | 5    | 4.9  | 6.1  | 5          |
| Yield (in percent)          | 70.5       | 75    | 74    | 74    | 73.4       | 60.3       | 62.5 | 61.4       | 62   | 59  | 62.5            | 62.5 | 58   | 60.8       | 46.5 | 45.8               | 46.5 | 45.5 | 48.8 | 46.6       |
| Defibering properties       | Fair       |       |       |       |            | Very good  |      |            |      |     | Very good       |      |      |            |      | Already comminuted |      |      |      |            |
| Appearance of material      | White      |       |       |       |            | White      |      |            |      |     | Yellowish-white |      |      |            |      | Bright yellow      |      |      |      |            |
| Fibre structure             | Maintained |       |       |       |            | Maintained |      |            |      |     | Maintained      |      |      |            |      | Destroyed          |      |      |      |            |
| pH (of spent liquor)        | 1.7        | 1.8   | 1.6   | 1.7   | 1.7        | 1.6        | 1.8  | 1.7        | 1.5  | 1.6 | 1.7             | 1.6  | 1.5  | 1.6        | 1.4  | 1.5                | 1.6  | 1.5  | 1.7  | 1.5        |

Comparison of these results with those obtained in Example III (Table 3), using nitrogen above the liquor, shows that at 200° C. approximately the same yield is obtained in 1½ to 2 hours as is obtained after 10 hours at 150° C., while the lignin contents of the products do not differ greatly. Extension of the cooking time to 2½ hours reduces the D.P. considerably at this temperature. Accordingly, at 200° C. digestion times of 1½ to 2 hours or a period not greatly in excess of 2 hours may be used.

Trials were further carried out using above the digestion liquor nitrogen containing 2%, 5% and 10% of oxygen. The reaction conditions were 200° C., together with mechanical treatment throughout the digestion, i.e. the conditions were as severe as possible. With 2% of oxygen in the nitrogen gas the color of the product and of the spent liquor was very similar to the case when nitrogen alone was used above the reaction liquor. Using 5% of oxygen in the gas, there was a slight browning of the material while with 10% of oxygen in the gas the cooking liquor blackened considerably and in addition the material itself darkened. These trials demonstrate that at above 5% of oxygen in the inert gas there is a tendency to darken both in the liquor and in the material itself.

#### EXAMPLE V

This example demonstrates that if the chips are wholly submerged in the liquor throughout the digestion process then results are obtained very similar to those using normal digestion conditions but having nitrogen or other inert gas above the liquor. The cooking liquor and other conditions were the same as those in Example II with the exception that trials were carried out both with and without simultaneous grinding, and to ensure complete submersion of the chips the ratio of chips to liquor was 1:21. The results obtained were as follows:

Table 5

| Trial number.....                | With<br>grind-<br>ing | Without grinding |       |       |       |       |
|----------------------------------|-----------------------|------------------|-------|-------|-------|-------|
|                                  |                       | M 30             | 3     | 4     | 6     | 6a    |
| D.P.....                         | 1,186                 | 1,950            | 2,040 | 2,053 | 1,955 | 2,009 |
| Lignin content (in percent)..... | 10                    | 13.7             | 14    | 14.5  | 13.9  | 14    |
| Yield (in percent).....          | 59.6                  | 69               | 70    | 71    | 70    | 70    |
| Defibering properties            | Very good             | Fair             | Fair  | Fair  | Fair  |       |
| Appearance of material           | White                 | Yellowish-white  |       |       |       |       |
| Fiber structure.....             | Maintained            | Maintained       |       |       |       |       |

I claim:

1. A process for the production of pulps from lignin-containing cellulosic material, which consists in simultaneously subjecting the cellulosic material to mechanical disintegration and to digestion with an acid sulfite cooking liquor without previous impregnation with said liquor, under an atmosphere which consists, in addition to constituents evaporated from the liquor itself, of inert gas containing not more than 5% of oxygen.
2. A process for the production of pulps from lignin-containing cellulosic material, which consists in simul-

taneously subjecting the cellulosic material to mechanical disintegration and to digestion with an acid sulfite cooking liquor without previous impregnation with said liquor, under an atmosphere which consists, in addition to constituents evaporated from the liquor itself, of inert gas containing not more than 5% of oxygen, in a closed digestor and under the autogenous pressure developed in the digestor at the digesting temperature.

3. A process for the production of pulp from lignin-containing cellulosic material, which comprises simultaneously subjecting the cellulosic material to mechanical disintegration and to digestion with an acid sulfite cooking liquor at a temperature between 150° and 200° C., without previous impregnation with said liquor, under an atmosphere which consists, in addition to constituents evaporated from the liquor itself, of inert gas containing not more than 5% of oxygen.

4. A process for the production of pulps from lignin-containing cellulosic material, which consists in simultaneously subjecting the cellulosic material to mechanical disintegration and to digestion with an acid sulfite cooking liquor without previous impregnation with said liquor, under an atmosphere which consists, in addition to constituents evaporated from the liquor itself, of inert gas containing not more than 2% of oxygen.

5. A process for the production of pulps from lignin-containing cellulosic material, which consists in simultaneously subjecting the cellulosic material to mechanical disintegration and to digestion with an acid sulfite cooking liquor without previous impregnation with said liquor, under an atmosphere which consists, in addition to constituents evaporated from the liquor itself, of substantially pure nitrogen.

6. A process for the production of pulps from lignin-containing cellulosic material, which consists in simultaneously subjecting the cellulosic material to mechanical disintegration and to digestion with an acid sulfite cooking liquor without previous impregnation with said liquor, under an atmosphere which consists, in addition to constituents evaporated from the liquor itself, of carbon dioxide.

7. A process for the production of pulps from lignin-containing cellulosic material, which consists in simultaneously subjecting the cellulosic material to mechanical disintegration and to digestion with an acid sulfite cooking liquor containing a bisulfite whose cation is selected from the group consisting of sodium, potassium, ammonium, calcium, and magnesium and which contains free sulphur dioxide, the digestion being carried out without previous impregnation with said liquor and under an atmosphere which consists, in addition to constituents evaporated from the liquor itself, of inert gas containing not more than 5% of oxygen.

55 References Cited in the file of this patent

UNITED STATES PATENTS

1,587,631 Clark ..... June 8, 1926  
1,903,962 Dreyfus ..... Apr. 18, 1933

60 FOREIGN PATENTS

201,259 Germany ..... Jan. 5, 1907

OTHER REFERENCES

65 Scheller: The Influence of Elementary and Active Oxygen on Cellulose on the Basis of Viscosity Measurements, TAPPI Series XXV, pages 551-555, June 1942.